

Patented July 15, 1924.

1,501,383

# UNITED STATES PATENT OFFICE.

DALY O. WHITE, OF PORTLAND, MAINE

## MOTOR FUEL.

No Drawing.

Application filed September 28, 1923. Serial No. 665,455.

To all whom it may concern:

Be it known that I, DALY O. WHITE, residing at 6 Horton Place, in the city of Portland, county of Cumberland, and State 5 of Maine, have invented new and useful Improvements in Motor Fuels, of which the following is a specification.

The present invention pertains to a new fuel especially adapted for use in gasoline 10 engines.

The fuel consists of ethyl alcohol to which are added wood alcohol, sal ammoniac, phenol, and a small quantity of ether.

These additions to the ethyl alcohol each 15 have an independent effect, and as few or as many of them as desired may be used. In other words, one or more of these additions may be employed in the absence of the remaining ones, according to the properties 20 desired in the resulting mixture. The function of the wood or methyl alcohol is merely to denaturize the ethyl alcohol as required by law. The sal ammoniac acts as a decarbonizing agent in the cylinders and therefore 25 constitutes one of the more important ingredients. The phenol has a similar effect especially in removing hard particles of metal and dirt which may find their way to the cylinders. A small addition of ether 30 renders the mixture more explosive.

It has been found that the following combinations, some of which are compounded with a view to omit some of the properties above mentioned, result in satisfactory mixtures. The term "alcohol" implies ethyl 35 alcohol alone, or a mixture of ethyl alcohol with sufficient methyl alcohol for denaturizing. The combinations are as follows:

1. 98% ethyl alcohol, 2% ether.
2. 98% alcohol, 1.75% ether, .25%  $\text{NH}_4\text{Cl}$ .
3. 98% alcohol, 1.75% ether, .125%  $\text{NH}_4\text{Cl}$ , .125% phenol.
4. 99.5% alcohol, .5%  $\text{NH}_4\text{Cl}$ .

In the use of this fuel it is found possible 45 to obtain an unusually high efficiency because of two sets of factors:

I. The greater ease with which complete combustion can be obtained, and the smaller proportion of air needed as compared with 50 the quantity of air needed to mix with gasoline.

II. The fact that with this fuel far higher compression and a much cooler cycle are obtained.

55 In considering the first question of combustion, it is known that a good gasoline may

for all practical purposes be regarded as hexane  $\text{C}_6\text{H}_{14}$ , as it is a mixture of this with the lower and the next higher members of the group in proportions which give about 60 this composition. The complete combustion of this compound may be represented.



so that 2 volumes of hydrocarbon require 19 volumes of oxygen. Since oxygen constitutes 20.9% of the atmosphere, we can take the amount of air required as

$$\frac{100 \times 19}{20.9} = 90.9$$

or 1 volume will require 45.45 volumes of air. In a gasoline motor this would mean that for complete combustion there should 75 be no more than 21% of gasoline vapor in the mixture entering the combustion chamber. Since practice has led to generally 1½ times the theoretical proportion of air being admitted, the gasoline vapor is diluted 80 with about 68 times its volume of air, four-fifths of which is inert nitrogen taking no part in the reaction but tending to hinder and retard the combustion. Indeed, under ordinary pressure such a mixture would not 85 burn, much less explode.

The compression of this mixture before explosion can be taken to be about 80 lbs. per square inch, owing to the risk of premature ignition. The explosion then takes 90 place with such rapidity that the diluting action of the nitrogen present prevents complete combustion. The results of the incomplete combustion thus caused are the low efficiency, stench, and deposit of carbon 95 which now attend the operation of a gasoline motor.

Compounds like the members of the paraffin group which go to form gasoline are 100 highly susceptible to changes from rise of temperature, and the heat generated by the compression already brings about a certain amount of change. It is known that a temperature of about  $1200^\circ \text{C}$ . is needed to ignite the ordinary gasoline and air mixture at atmospheric pressure. At the moment of explosion, such portions of the hydrocarbon as do not happen to be in contact with the proper quantity of oxygen required for their combustion, owing to the hindering action 105 of the inert hydrogen, undergo changes of various complexity. The result is that the

products of combustion contain not only the products of complete combustion but also the products of incomplete combustion such as carbon monoxide and considerable quantities of hydrocarbon such as ethane, propane and acetylene. These are formed by the heat at the moment of explosion, and it is these products combined with the lubricants that give not only the odors now associated with gasoline motors, but aid also in depositing a film of carbon on the inside of the cylinders.

With the above mentioned new solution containing alcohol as a base, there does not occur the same difficulty in obtaining complete combustion when once the mixture of vapor and air is made. The reaction is



so that the air required will be

$$\frac{100 \times 3}{20.9} = 14.3 \text{ vols.}$$

per volume of alcohol vapor, or roughly one-third the amount of air needed with gasoline. It is fairly easy with this more moderate proportion of air to attain an approximation to complete combustion, more especially because double the compression possible with gasoline can be used.

The combustion is largely dependent upon the existing temperature and the use of methyl alcohol tends to result in the formation of acetic products which have a more or less corrosive effect on the valves and metal work. This difficulty is offset in the new solution by the addition of the ammonium chloride which forms ammonium acetate with the acetyl products and also forms muriatic acid. The ammonium acetate has no effect on the inside of the cylinder or the metal parts, and the little muriatic acid formed there would have a tendency to keep the cylinder clean and free from any particles of carbon which might adhere to the sides of the cylinder. It has been found that automobiles of all makes, after having this solution used in them for a period of three or more weeks, showed no tendency towards corrosion in any manner.

The alcohol is carburetted with ether which has a tendency to give the mixture a greater range of explosive power. Phenol is added to the solution and not only increases the power obtained but also keeps the inside of the cylinders free and clear from any particles of dirt which might adhere to the cylinder walls. It has been found that

an increased amount of phenol tends to make the solution more miscible in all proportions and gives a much better cycle in the motor. The phenol also has a tendency to absorb the muriatic acid and form  $\text{C}_6\text{H}_5\text{Cl}$  and  $\text{H}_2\text{O}$ , thereby leaving little or possibly no  $\text{HCl}$  in the cylinders.

An added advantage is due to the relatively cool cycle, which requires less oil and consequently decreases the tendency to form carbon.

The advantages in full can be summed up as follows:

- I. A comparatively cool cycle.
- II. More mileage per gallon of fuel.
- III. Less consumption of oil.
- IV. More power.
- V. Noncarbonizing.
- VI. The possibility of adding the mixture to gasoline in all proportions.

In further explanation of the last consideration, it is pointed out that the advantages of this mixture may be realized in proportion to the amount of mixture used as an addition to gasoline, the ratio between the amount of the mixture and the amount of the gasoline being determined by the construction of the motor and the conditions of operation.

The proportions cited in the specification and claims are those which have been found by me to give the most satisfactory results. It will be understood that variations in these proportions may be made within reasonable limits without departing from the spirit of the invention. The result of such variations will consist only in the realization to a greater or less degree of the properties ascribed to the particular ingredients, but will not give rise to a principle of operation different from that described.

Having thus fully described the invention, what I claim as new and desire to protect by Letters Patent is:—

1. A fuel composed of alcohol and a relatively small addition of  $\text{NH}_4\text{Cl}$ .
2. A fuel composed of grain alcohol and relatively small additions of wood alcohol and  $\text{NH}_4\text{Cl}$ .
3. A fuel composed of alcohol and .5%  $\text{NH}_4\text{Cl}$ .
4. A fuel consisting of 98% alcohol, 1.75% ether, and .25%  $\text{NH}_4\text{Cl}$ .
5. A fuel consisting of 98% alcohol, 1.75% ether, .125%  $\text{NH}_4\text{Cl}$ , and .125% phenol.

In witness whereof I have hereunto set my hand.

DALY O. WHITE.